# EUROPEAN PATENT SPECIFICATION

(11) **EP 4 066 964 B1**
(45) Date of publication and mention of the grant of the patent: **04.10.2023**
(21) Application number: 21202284.2
(22) Date of filing: 12.10.2021
(51) Int. Cl.: B22F 1/142, B22F 9/04, C21C 7/072, C21C 7/10, C21D 1/26, C21D 1/74, C21D 6/00, C22C 33/02, C22C 33/04, C22C 38/00, H01F 1/057, H01F 41/02

(54) **METHOD FOR PREPARING A HIGH-PERFORMANCE ND-FE-B ISOTROPIC MAGNETIC POWDER**
VERFAHREN ZUR HERSTELLUNG EINES HOCHLEISTUNGSFÄHIGEN ISOTROPEN ND-FE-B-MAGNETPULVERS
PROCÉDÉ DE PRÉPARATION D'UNE POUDRE MAGNÉTIQUE ISOTROPE ND-FE-B HAUTE PERFORMANCE

(30) Priority: 01.04.2021 CN 202110356690
(43) Date of publication of application: 05.10.2022
(73) Proprietor: Baotou Kerui Micro Magnet New Materials Co., Ltd., Baotou, Inner Mongolia 014030 (CN)
(72) Inventor: LIN, Jirong, Baotou, 014030 (CN); WANG, Ruigang, Baotou, 014030 (CN); WANG, Zhigang, Baotou, 014030 (CN); REN, Jianxin, Baotou, 014030 (CN)
(74) Representative: Kordel, Mattias

(56) References cited:
- CN-A- 102 990 057
- CN-A- 106 486 227
- CN-A- 110 660 553
- JP-A- H10 130 796
- US-A1- 2002 117 235

## Description

### TECHNICAL FIELD

The present invention relates to a method for preparing a high-performance Nd-Fe-B isotropic magnetic powder.

### BACKGROUND ART

Neodymium-iron-boron (Nd-Fe-B) rare earth magnetic materials could be essentially divided into two types according to the production process. One is sintered Nd-Fe-B, and the other is isotropic Nd-Fe-B. The basic raw material of isotropic Nd-Fe-B magnet is called Nd-Fe-B rapidly-quenched magnetic powder. The large-scale production and application of rapidly-quenched magnetic powder began in the late 1980s. The basic raw materials of the Nd-Fe-B rapidly-quenched magnetic powder are rare earth metals praseodymium and neodymium, boron, and metal iron. The production process of rapidly-quenched magnetic powder is very complex, mainly including smelting, rapidly quenching, crushing to magnetic powder and crystallizing the magnetic powder, etc.

The development and research in this field in China has a history of more than 20 years, but for the above reasons, there is no final breakthrough in key technologies, especially in how to control the rapid solidification rate of molten alloy, and the progress is slow. Therefore, a small-scale production has been achieved in a few domestic manufacturers; however, they do not have the capacity to produce high-performance magnetic on a large scale.

The applicant has been researching and developing various production processes of high-performance Nd-Fe-B rapidly-quenched magnetic powder. Through a large number of experimental studies, it has been found that even if a powerful vacuum unit is used to keep the rapid quenching furnace in a high vacuum state, the obtained magnetic powder still has very high oxygen content, and thereby the magnetic performance of the magnetic powder is not high. Further, it has been found that in the high vacuum state, materials such as vacuum furnace wall and crucible would continuously release a large amount of water vapor, oxygen, and nitrogen at high temperature, and these impurity gases would have a great opportunity to oxidize high-temperature Nd-Fe-B in the nozzle and crucible before being discharged, thereby improving the oxygen content of magnetic powder, destroying the lattice structure of Nd-Fe-B, and reducing the magnetic performance of magnetic powder. Therefore, how to reduce the oxygen content in magnetic powder is one of the important ways to produce high-performance magnetic powder.

For example, CN103862052A discloses a forming method of isotropic Nd-Fe-B magnet. The method includes the steps of smelting raw materials into a pre-alloyed ingot, amorphizing the pre-alloyed ingot to obtain a rapidly-quenched alloy, ball milling the rapidly-quenched alloy to obtain a powder, mixing the powder with a binder to form a slurry, and forming the slurry into a magnet, and further includes the step of treating the powder surface with a surface treatment agent, which could reduce the oxygen content of isotropic Nd-Fe-B.

CN111755237A discloses a Nd-Fe-B magnet and a method for regulating the grain size and particle size distribution of the coarse-grained layer of the Nd-Fe-B magnet. In the method, the Nd-Fe-B rapidly-quenched magnetic powder was pickled with an acidic solution, washed and dried to reduce the oxygen content on the surface of the Nd-Fe-B rapidly-quenched magnetic powder by at least 200 ppm. The rapidly-quenched magnetic powder prepared by this method makes it possible to improve the coercivity of isotropic Nd-Fe-B magnet and anisotropic Nd-Fe-B magnet.

CN106486227A discloses a lanthanum cerium iron-based permanent magnet powder, with a chemical formula as follows: (CeₓLa_{y}Re_{100-x-y})ₐFe_{100-a-b-c}B_{b}TM_{c}, wherein, a, b, and c respectively represent a mass percentage of corresponding atom; 26%≤a≤30%, 0.8%≤b≤1.2%, and 0%≤c≤5%; Re is one or more selected from the group consisting of Pr, Nd, Sm, Gd, Tb, Dy, Ho, Er, Yb, and Lu; and TM is one or more selected from the group consisting of Ga, Co, Cu, Nb, Al, and Zr.

CN110660553A discloses an isotropic hot-pressed NdFeB magnetic powder, with a chemical formula as follows: (Nd_{1-w-x}Pr_{w}Dyₓ)_{α}(Fe_{1-y-z}Co_{y}Ga_{z})_{100-α-β}B_{β}; wherein α is any number between 12 and 16; β is any number between 4 and 7; x is any number between 0 and 0.2; y is any number between 0 and 0.1; z is any number between 0 and 0.01; w is any number between 0 and 1; and the unit is atomic ratio.

JPH10130796A discloses a compound with a chemical formula as follows: Fe_{100-x-y}BₓR_{y}, wherein R is one or more selected from the group consisting of Pr, Nd, and Dy.

US20020117235A1 discloses a method of making a material alloy for an iron-based rare earth magnet, the method comprising the steps of: preparing a melt of an iron-based rare earth material alloy, the material alloy having a composition represented by the general formula: (Fe₁₋ₘTₘ)_{1-00-x-y-z-n}(B₁₋ₚCₚ)ₓR_{y}Ti_{z}Mₙ, where T is at least one element selected from the group consisting of Co and Ni; R is at least one element selected from the group consisting of Y and the rare earth elements; and M is at least one element selected from the group consisting of Al, Si, V, Cr, Mn, Cu, Zn, Ga, Zr, Nb, Mo, Ag, Hf, Ta, W, Pt, Au and Pb; the mole fractions x, y, z, m, n and p satisfying the inequalities of: 10 at %<x≤25 at %; 6 at %≤y<10 at %; 0.5 at %≤z≤12 at %; 0≤m≤0.5; 0at %≤n≤10 at %; and 0≤p≤0.25, respectively; feeding the melt of the material alloy onto a guide having a guide surface that defines an angle of about 1 degree to about 80 degrees with respect to a horizontal plane so as to move the melt onto a region where the melt comes into contact with a chill roller; and rapidly cooling the melt using the chill roller to make a rapidly solidified alloy comprising an R₂Fe₁₄B phase.

CN102990057A discloses a method for producing a high-performance NdFeB bonded magnetic powder, comprising: dividing rapidly quenched magnetic powders into three categories: over-quenched magnetic powder, under-quenched magnetic powder, and reasonable quenched magnetic powder according to the difference of crystal microstructure and crystal average size of the magnetic powder; and heat-treating the divided magnetic powders with different temperature and time.

Although the above existing technologies could reduce the oxygen content to a certain extent by a surface treatment of rapidly-quenched magnetic powder, the effect is not good. In addition, the existing production process needs to be improved and the operation cost is high, so it is impossible to popularize on a large scale.

### SUMMARY

In order to solve the above technical problems, the present invention provides a method for preparing a high-performance neodymium-iron-boron isotropic magnetic powder. The method allows effectively reducing the oxygen content by controlling parameters such as the pressure value and flow rate of the inert gas in the rapid quenching furnace. Thus the prepared rapidly-quenched magnetic powder exhibits improved performance by not less than 10% than the same kind of magnetic powder.

In order to achieve the above object, the present invention provides the following technical solutions:

The present invention provides a method for preparing a high-performance neodymium-iron-boron isotropic magnetic powder, comprising the following steps:
S1, smelting alloy
   smelting and refining ingredients under vacuum to obtain an alloy ingot, and crushing the alloy ingot to obtain an alloy block,
   wherein the smelting is conducted at a temperature of 1,350-1,450 °C, and the refining is conducted at a temperature of 1,335-1,430 °C and a pressure of 900-1,100 Pa in an inert gas atmosphere for 3-7 minutes;
S2, rapidly quenching alloy solution
   melting the alloy block obtained in step S1 to obtain an alloy solution, rapidly quenching the alloy solution to form a Nd-Fe-B rapidly-quenched alloy plate;
S3, crushing alloy plate
   crushing the Nd-Fe-B rapidly-quenched alloy plate obtained in step S2 to obtain a magnetic powder; and
S4, crystallization heat treatment
   subjecting the magnetic powder obtained in step S3 to a crystallization heat treatment in an inert gas atmosphere, and cooling to obtain the Nd-Fe-B isotropic magnetic powder;
      wherein
      rapidly quenching the alloy solution in S2 is conducted under conditions: charging argon gas through a vacuum ball valve, maintaining a charging rate of argon gas of 0.2-1.5 m³/min; adjusting a vacuum butterfly valve, and maintaining a pressure of 200-2,000 Pa;
      the inert gas in steps S1 and S4 is argon gas; and
   the ingredients consisted of the following ingredients, in percentages by weight, 26.2% of rare earth metals praseodymium and neodymium, 4.7% of boron iron, 0.2% of metal niobium, 2.0% of metal cobalt, and the balance of ingot iron; the rare earth metals praseodymium and neodymium have a purity of 99.9%, in which the oxygen content is less than 400 ppm and the nitrogen content is less than 60 ppm; the ingot iron has a carbon content of less than 400 ppm, and a silicon content of less than 1,500 ppm; the boron iron has a boron content of 20.2%; the metal niobium has a purity of 99.5%; the metal cobalt has a purity of 99.9%, in which the oxygen content is less than 500 ppm, and the nitrogen content is less than 70 ppm.

In some embodiments, the smelting in step S1 is conducted at a temperature of 1,395 °C. In some embodiments, the refining is conducted at 1,380 °C and 1,000 Pa in an argon gas atmosphere for 5 minutes.

In some embodiments, the alloy block in step S1 has a particle size of 10-50 mm, and preferably 15-45 mm. The particle size of the alloy block is determined with screens having different pore diameters. For example, the alloy block could pass through the screen having a pore diameter of 50 mm, but could not pass through the screen having a pore diameter of 10 mm.

In some embodiments, rapidly quenching the alloy solution in step S2 is conducted under conditions: controlling a charging flow rate of the inert gas of 0.4-1.0 m³/min, and maintaining a pressure of 400-1,900 Pa.

In some embodiments, the magnetic powder in step S3 has a particle size of 45-380 µm, and preferably 58-250 µm. The particle size of the magnetic powder is determined with screens having different pore diameters. For example, the magnetic powder could pass through the screen having a pore diameter of 380 µm, but could not pass through the screen having a pore diameter of 45 µm.

In some embodiments, the crystallization heat treatment in step S4 is conducted at a temperature of 630-700 °C for 9-18 min, and preferably at a temperature of 650-680 °C for 10-15 min.

The technical solutions according to the present invention has the following beneficial effects:
(1) The present invention allows effectively reducing the oxygen content of the magnetic powder and improving the magnetic performance of the rapidly-quenched magnetic powder by improving the parameters such as alloy smelting, refining, and pressure and flow rate of the inert gas in the rapid quenching furnace.
(2) In the present invention, there is no need to modify the existing process equipment, and meanwhile there is no need to use additional organic reagents. Therefore, the method is low in operation cost, greener and more environmentally friendly, and thus is suitable for large-scale promotion and application.

### DETAILED DESCRIPTION OF THE EMBODIMENTS

The description of the following embodiments is only used to help understand the method and the core idea of the present invention. The following description of the disclosed embodiments enables those skilled in the art to implement or use the present invention.

Unless otherwise defined, all technical and scientific terms used herein have the same meaning as commonly understood by those of ordinary skill in the technical field to which the present disclosure belongs.

The ingredients used in examples of the present invention consisted of the following ingredients, in percentages by weight, 26.2% of rare earth metals praseodymium and neodymium, 4.7% of boron iron, 0.2% of metal niobium, 2.0% of metal cobalt, and the balance of ingot iron. The rare earth metals praseodymium and neodymium had a purity of 99.9%, in which the oxygen content was less than 400 ppm and the nitrogen content was less than 60 ppm. The ingot iron had a carbon content of less than 400 ppm, and a silicon content of less than 1,500 ppm. The boron iron had a boron content of 20.2%. The metal niobium had a purity of 99.5%. The metal cobalt had a purity of 99.9%, in which the oxygen content was less than 500 ppm, and the nitrogen content was less than 70 ppm.

### Basic Example A high-performance neodymium-iron-boron isotropic magnetic powder and its preparation method

The high-performance neodymium-iron-boron isotropic magnetic powder was prepared according to the following steps:

### S1. smelting alloy

Ingredients were added into an intermediate frequency vacuum induction furnace, smelted and refined therein, and cast into an alloy ingot. The alloy ingot was crushed, obtaining an alloy block with a particle size of 10-50 mm.

The smelting was conducted at a temperature of 1,350-1,450 °C. The refining was conducted at a temperature of 1,335-1,430 °C and a pressure of 900-1,100 Pa in an inert gas atmosphere for 3-7 minutes.

### S2. rapidly quenching alloy solution

The alloy block obtained in step S1 was added to a vacuum induction melting-rapid quenching furnace, and molten therein, obtaining an alloy solution. The alloy solution was rapidly quenched into a Nd-Fe-B rapidly-quenched alloy plate.

Rapidly quenching the alloy solution was conducted under conditions: charging argon gas through a vacuum ball valve, maintaining a charging rate of argon gas of 0.2-1.5 m³/min; adjusting a vacuum butterfly valve, and maintaining a pressure of 200-2,000 Pa

### S3. crushing alloy plate

The Nd-Fe-B rapidly-quenched alloy plate obtained in step S2 was crushed, obtaining a magnetic powder with a particle size of 45-380 µm.

### S4. crystallization heat treatment

The magnetic powder obtained in step S3 was subjected to a crystallization heat treatment in an argon gas atmosphere, and cooled, obtaining the neodymium-iron-boron isotropic magnetic powder.

The crystallization heat treatment was conducted at a temperature of 630-700 °C for 9-18 min.

### Examples 1-5 A high-performance neodymium-iron-boron isotropic magnetic powder and its preparation method

The process parameters in the methods for preparing the high-performance Nd-Fe-B isotropic magnetic powders are shown in Table 1.

**Table 1**

| Parameters | Example 1 | Example 2 | Example 3 | Example 4 | Example 5 |
|---|---|---|---|---|---|
| Temperature for smelting /°C | 1350 | 1450 | 1395 | 1395 | 1395 |
| Temperature for refining /°C | 1335 | 1430 | 1380 | 1380 | 1380 |
| Pressure for refining /Pa | 1100 | 900 | 1000 | 1000 | 1000 |
| Time for refining /min | 7 | 3 | 5 | 5 | 5 |
| Particle size of the alloy block /mm | 10 | 50 | 15 | 45 | 30 |
| Charging flow rate of argon gas /(m³/min) | 0.2 | 1.5 | 0.4 | 1.0 | 0.6 |
| Pressure /Pa | 200 | 2000 | 800 | 1900 | 1330 |
| Particle size of the magnetic powder /µm | 380 | 45 | 58 | 250 | 200 |
| Temperature for crystallization heat treatment /°C | 630 | 700 | 650 | 680 | 665 |
| Time /min | 18 | 9 | 15 | 10 | 13 |

### Comparative Example 1 A neodymium-iron-boron isotropic magnetic powder and its preparation method

This comparative example was performed according to the method as described in Example 5, expect that rapidly quenching alloy solution in step S2 was conducted under conditions: a vacuum degree in the vacuum induction melting-rapid quenching furnace was 2×10⁻² Pa, and argon gas was not charged.

### Comparative Example 2 A neodymium-iron-boron isotropic magnetic powder and its preparation method

This comparative example was performed according to the method as described in Example 5, expect that rapidly quenching alloy solution in step S2 was conducted under conditions: argon gas was charged through a vacuum ball valve to a pressure of 1,330 Pa, and the exhaust vacuum butterfly valve was closed.

### Comparative Example 3 A neodymium-iron-boron isotropic magnetic powder and its preparation method

This comparative example was performed according to the method as described in Example 5, expect that argon gas was charged through a vacuum ball valve to a pressure of 3,000 Pa, and the exhaust vacuum butterfly valve was closed.

### [ Comparative Example 4 A neodymium-iron-boron isotropic magnetic powder and its preparation method

The high-performance neodymium-iron-boron isotropic magnetic powder was prepared according to the following steps:

### S1. smelting alloy

Ingredients were added into an intermediate frequency vacuum induction furnace, smelted and refined therein, and cast into an alloy ingot. The alloy ingot was crushed, obtaining an alloy block with a particle size of 40 mm.

The smelting was conducted at a temperature of 1,500 °C. The refining was conducted at a temperature of 1,450 °C and a pressure of 200 Pa in an inert gas atmosphere for 25 minutes.

### S2. rapidly quenching alloy solution

The alloy block obtained in step S1 was added to a vacuum induction melting-rapid quenching furnace, and molten therein, obtaining an alloy solution. The alloy solution was rapidly quenched into a Nd-Fe-B rapidly-quenched alloy plate.

Rapidly quenching the alloy solution was conducted under conditions: charging argon gas through a vacuum ball valve, maintaining a charging flow rate of argon gas of 3 m³/min; adjusting a vacuum butterfly valve, and maintaining a pressure of 2,500 Pa.

### S3. crushing alloy plate

The Nd-Fe-B rapidly-quenched alloy plate obtained in step S2 was crushed, obtaining a magnetic powder with a particle size of 200 µm.

### S4. crystallization heat treatment

The magnetic powder obtained in step S3 was subjected to a crystallization heat treatment in an argon gas atmosphere, and cooled, obtaining the neodymium-iron-boron isotropic magnetic powder.

The crystallization heat treatment was conducted at 720 °C for 10 min.

### Comparative Example 5 A neodymium-iron-boron isotropic magnetic powder and its preparation method

The high-performance neodymium-iron-boron isotropic magnetic powder was prepared according to the following steps:

### S1. smelting alloy

Ingredients were added into an intermediate frequency vacuum induction furnace, smelted and refined therein, and cast into an alloy ingot. The alloy ingot was crushed, obtaining an alloy block with a particle size of 40 mm.

The smelting was conducted at 1,300 °C. The refining was conducted at a temperature of 1,285 °C and a pressure of 1,500 Pa in an inert gas atmosphere for 10 minutes.

### S2. rapidly quenching alloy solution

The alloy block obtained in step S1 was added to a vacuum induction melting-rapid quenching furnace, and molten therein, obtaining an alloy solution. The alloy solution was rapidly quenched into a Nd-Fe-B rapidly-quenched alloy plate.

Rapidly quenching the alloy solution was conducted under conditions: charging argon gas through a vacuum ball valve, maintaining a charging flow rate of argon gas of 0.1 m³/min; adjusting a vacuum butterfly valve, and maintaining a pressure of 80 Pa.

### S3. crushing alloy plate

The Nd-Fe-B rapidly-quenched alloy plate obtained in step S2 was crushed, obtaining a magnetic powder with a particle size of 200 µm.

### S4. crystallization heat treatment

The magnetic powder obtained in step S3 was subjected to a crystallization heat treatment in an argon atmosphere, and cooled, obtaining the neodymium-iron-boron isotropic magnetic powder.

The crystallization heat treatment was conducted at 600 °C for 20 min.

The neodymium-iron-boron isotropic magnetic powders prepared in Examples 1-5 and Comparative Examples 1-5 were subjected to an oxygen content analysis and a magnetic performance analysis (VSM measurement). The results are shown in Table 2.

**Table 2 Magnetic performance of neodymium-iron-boron isotropic magnetic powders**

| | Oxygen content% | Br (kGs) | Hci (kOe) | BHₘₐₓ (MGoe) |
|---|---|---|---|---|
| Example 1 | 0.09 | 8.69 | 9.32 | 14.4 |
| Example 2 | 0.02 | 8.70 | 9.63 | 14.6 |
| Example 3 | 0.07 | 8.71 | 9.50 | 14.8 |
| Example 4 | 0.02 | 8.72 | 9.56 | 14.9 |
| Example 5 | 0.02 | 8.79 | 9.62 | 15.7 |
| Comparative Example 1 | 0.21 | 8.57 | 9.06 | 13.6 |
| Comparative Example 2 | 0.15 | 8.62 | 9.24 | 13.9 |
| Comparative Example 3 | 0.13 | 8.61 | 9.26 | 14.1 |
| Comparative Example 4 | 0.11 | 8.63 | 9.25 | 14.2 |
| Comparative Example 5 | 0.14 | 8.59 | 9.21 | 13.8 |

The applicant found that under high vacuum conditions, when oxygen molecules appeared in the rapid quenching furnace due to various reasons, its mean free path would be very long. For example, at a vacuum degree of 1.33×10⁻² Pa, the mean free path of oxygen molecules under ideal conditions is 0.52 m. That is to say, oxygen molecule, with an average velocity of 450 m/s, once appears in the vacuum furnace, it has enough chances to reach the neodymium-iron-boron stream or the surface of the liquid in the crucible below the nozzle, and react with neodymium atoms in the neodymium-iron-boron, before being pumped away by the vacuum unit. This is the reason why the oxygen content in the magnetic powder could not be reduced by using high vacuum means.

Meanwhile, the applicant found that if a small amount of argon gas was charged and retained in the rapid quenching furnace, when the pressure reached 133 Pa, the mean free path of oxygen molecules would rapidly drop to 0.052 mm, and when the pressure of argon gas in the rapid quenching furnace reached 2,000 Pa, the mean free path of oxygen atoms at the same temperature would drop to 2.0 µm or less. Argon gas forms a complete protective layer around the neodymium-iron-boron liquid. At this time, the frequency of collisions between gas molecules reached 70 million times per second! Therefore, if oxygen atoms appear in the rapid quenching furnace, most of the oxygen atoms would be discharged from the rapid quenching furnace by the vacuum pump before they have a chance to reach the surface of the Nd-Fe-B liquid. By continuously charging argon gas while discharging the contaminated argon gas by a vacuum pump, harmful molecules such as water vapor, oxygen, and nitrogen are carried away, which could effectively reduce the amount of harmful molecules such as water vapor, oxygen, and nitrogen in the rapid quenching furnace.

After a series of tests and studies, it is shown that if argon gas is continuously charged into the rapid quenching furnace meanwhile the gas in the furnace is continuously pumped off with a vacuum pump, and a continuous flow and exchange are maintained such that the pressure is maintained at 200 Pa or more, then the rapidly-quenched magnetic powder has a greatly reduced oxygen content. When the pressure of argon gas is 1,330 Pa, the magnetic powder has the lowest oxygen content. Also, experiments have proven that a better effect could be achieved when charging argon gas at the bottom of the furnace body and pumping off the gas and carrying away harmful gases at the top of the furnace body. However, the pressure in the furnace could not be too high, otherwise the oxygen content would no longer decrease due to the gas swirl caused by the highspeed rotation of the rapid quenching roll, and the gas swirl would also make the rapid quenching process more complicated and affect the magnetic performance.

In summary, the present invention allows effectively reducing the oxygen content of the magnetic powder and improving the magnetic performance of the rapidly-quenched magnetic powder by improving parameters such as the smelting, refining, and the pressure and flow rate of the inert gas in the rapid quenching furnace.

Also, in the present invention, there is no need to modify the existing process equipment, and there is no need to use additional organic reagents. The method is low in operation cost, greener and more environmentally friendly, and thus is suitable for large-scale promotion and application.

## Claims

1. A method for preparing a Nd-Fe-B isotropic magnetic powder, comprising
S1. smelting alloy
smelting and refining ingredients under vacuum to obtain an alloy ingot, and crushing the alloy ingot to obtain an alloy block,
wherein the smelting is conducted at a temperature of 1,350-1,450 °C, and the refining is conducted at a temperature of 1,335-1,430 °C and a pressure of 900-1,100 Pa in an inert gas atmosphere for 3-7 minutes;
S2. rapidly quenching alloy solution
melting the alloy block obtained in step S1 to obtain an alloy solution, rapidly quenching the alloy solution to form a Nd-Fe-B rapidly-quenched alloy plate;
S3. crushing alloy plate
crushing the Nd-Fe-B rapidly-quenched alloy plate obtained in step S2 to obtain a magnetic powder; and
S4. crystallization heat treatment
subjecting the magnetic powder obtained in step S3 to a crystallization heat treatment in an inert gas atmosphere, and cooling, to obtain the Nd-Fe-B isotropic magnetic powder;
wherein
rapidly quenching the alloy solution in S2 is conducted under conditions: charging argon gas through a vacuum ball valve, maintaining a charging rate of argon gas of 0.2-1.5 m³/min; adjusting a vacuum butterfly valve, and maintaining a pressure of 200-2,000 Pa;
the inert gas in steps S1 and S4 is argon gas; and
the ingredients consisted of the following ingredients, in percentages by weight, 26.2% of rare earth metals praseodymium and neodymium, 4.7% of boron iron, 0.2% of metal niobium, 2.0% of metal cobalt, and the balance of ingot iron; the rare earth metals praseodymium and neodymium have a purity of 99.9%, in which the oxygen content is less than 400 ppm and the nitrogen content is less than 60 ppm; the ingot iron has a carbon content of less than 400 ppm, and a silicon content of less than 1,500 ppm; the boron iron has a boron content of 20.2%; the metal niobium has a purity of 99.5%; the metal cobalt has a purity of 99.9%, in which the oxygen content is less than 500 ppm, and the nitrogen content is less than 70 ppm.

2. The method as claimed in claim 1, wherein the alloy block in step S1 has a particle size of 10-50 mm, as determined with screens.

3. The method as claimed in any one of claims 1 to 2, wherein rapidly quenching the alloy solution in step S2 is conducted under conditions: controlling a charging flow rate of the inert gas of 0.4-1.0 m³/min, and maintaining a pressure of 400-1,900 Pa.

4. The method as claimed in any one of claims 1 to 3, wherein the magnetic powder in step S3 has a particle size of 45-380 µm, as determined with screens.

5. The method as claimed in any one of claims 1 to 4, wherein the crystallization heat treatment in step S4 is conducted at a temperature of 630-700 °C for 9-18 min.

## Patentansprüche

1. Verfahren zur Herstellung eines isotropen magnetischen Nd-Fe-B-Pulvers, umfassend
S1. Schmelzen der Legierung
Schmelzen und Veredeln von Bestandteilen unter Vakuum, um einen Legierungsbarren zu erhalten, und Zerkleinern des Legierungsbarrens, um einen Legierungsblock zu erhalten,
wobei das Schmelzen bei einer Temperatur von 1.350 - 1.450 °C und das Veredeln bei einer Temperatur von 1.335 - 1.430 °C und einem Druck von 900 - 1.100 Pa in einer Inertgasatmosphäre für 3 - 7 Minuten durchgeführt wird;
S2. schnelles Quenchen der Legierungslösung
Schmelzen des in Schritt S1 erhaltenen Legierungsblocks, um eine Legierungslösung zu erhalten, schnelles Quenchen der Legierungslösung, um eine schnell gequenchte Nd-Fe-B-Legierungsplatte zu erzeugen;
S3. Zerkleinern der Legierungsplatte
Zerkleinern der in Schritt S2 erhaltenen schnell gequenchten Nd-Fe-B-Legierungsplatte, um ein magnetisches Pulver zu erhalten; und
S4. Kristallisationswärmebehandlung
Unterziehen des in Schritt S3 erhaltenen magnetischen Pulvers einer Kristallisationswärmebehandlung in einer Inertgasatmosphäre und Abkühlen, um das isotrope magnetische Nd-Fe-B-Pulver zu erhalten;
wobei
das schnelle Quenchen der Legierungslösung in S2 unter folgenden Bedingungen durchgeführt wird: Zuführen von Argongas durch ein Vakuumkugelventil, Aufrechterhalten einer Zuführungsrate von Argongas von 0,2 - 1,5 m³/min; Einstellen eines Vakuumabsperrventils, und Aufrechterhalten eines Drucks von 200 - 2.000 Pa;
das Inertgas in den Schritten S1 und S4 ist Argongas; und
die Bestandteile bestehen aus den folgenden Bestandteilen, in Gewichtsprozent, 26,2 % der Seltenerdmetalle Praseodym und Neodym, 4,7 % Bor-Eisen, 0,2 % des Metalls Niob, 2,0 % des Metalls Kobalt und der Rest aus Barreneisen; die Seltenerdmetalle Praseodym und Neodym haben eine Reinheit von 99,9 %, in denen der Sauerstoffgehalt weniger als 400 ppm und der Stickstoffgehalt weniger als 60 ppm beträgt; das Barreneisen hat einen Kohlenstoffgehalt von weniger als 400 ppm und einen Siliziumgehalt von weniger als 1.500 ppm; das Bor-Eisen hat einen Borgehalt von 20,2 %; das Metall Niob hat eine Reinheit von 99,5 %; das Metall Kobalt hat eine Reinheit von 99,9 %, in dem der Sauerstoffgehalt weniger als 500 ppm und der Stickstoffgehalt weniger als 70 ppm beträgt.

2. Verfahren nach Anspruch 1, wobei der Legierungsblock in Schritt S1 eine Teilchengröße von 10 - 50 mm aufweist, die mittels Sieben bestimmt wird.

3. Verfahren nach einem der Ansprüche 1 bis 2, wobei das schnelle Quenchen der Legierungslösung in Schritt S2 unter Bedingungen durchgeführt wird: Steuerung eines Zuführungsrate des Inertgases von 0,4 - 1,0 m³/min und Aufrechterhaltung eines Drucks von 400 - 1.900 Pa.

4. Verfahren nach einem der Ansprüche 1 bis 3, wobei das magnetische Pulver in Schritt S3 eine Partikelgröße von 45 - 380 pm hat, die mittels Sieben bestimmt wird.

5. Verfahren nach einem der Ansprüche 1 bis 4, wobei die Kristallisationswärmebehandlung in Schritt S4 bei einer Temperatur von 630 - 700 °C für 9 - 18 min durchgeführt wird.

## Revendications

1. Procédé de préparation d'une poudre magnétique isotrope de Nd-Fe-B, comprenant les étapes comprenant
S1. alliage de fusion
fondre et raffiner des ingrédients sous vide pour obtenir un lingot d'alliage, et broyer le lingot d'alliage pour obtenir un bloc d'alliage,
dans lequel la fusion est réalisée à une température de 1350-1450 °C, et le raffinage est réalisé à une température de 1335-1430 °C et une pression de 900-1100 Pa dans une atmosphère de gaz inerte pendant 3-7 minutes ;
S2. trempe rapide d'une solution d'alliage
faire fondre le bloc d'alliage obtenu dans l'étape S1 pour obtenir une solution d'alliage, effectuer une trempe rapide de la solution d'alliage pour former une plaque d'alliage de Nd-Fe-B ayant subi une trempe rapide ;
S3. broyage d'une plaque d'alliage
broyer la plaque d'alliage de Nd-Fe-B ayant subi une trempe rapide obtenue dans l'étape S2 pour obtenir une poudre magnétique ; et
S4. traitement thermique de cristallisation
soumettre la poudre magnétique obtenue dans l'étape S3 à un traitement thermique de cristallisation dans une atmosphère de gaz inerte, et refroidir, pour obtenir la poudre magnétique isotrope de Nd-Fe-B ;
dans lequel
la trempe rapide de la solution d'alliage dans S2 est réalisée dans des conditions de : introduction de gaz argon à travers une vanne à boisseau sphérique sous vide, maintien d'une vitesse d'introduction de gaz argon de 0,2-1,5 m3/min ; adaptation d'une vanne papillon sous vide, et maintien d'une pression de 200-2000 Pa ;
le gaz inerte dans les étapes S1 et S4 est du gaz argon ; et
les ingrédients consistaient en les ingrédients suivants, en pourcentages en poids, 26,2 % des métaux des terres rares praséodyme et néodyme, 4,7 % de ferrobore, 0,2 % de niobium métallique, 2,0 % de cobalt métallique, et pour le reste, du fer en lingot ; les métaux des terres rares praséodyme et néodyme ont une pureté de 99,9 %, dans laquelle la teneur en oxygène est inférieure à 400 ppm et la teneur en azote est inférieure à 60 ppm ; le fer en lingot a une teneur en carbone inférieure à 400 ppm, et une teneur en silicium inférieure à 1500 ppm ; le ferrobore a une teneur en bore de 20,2 % ; le niobium métallique a une pureté de 99,5 % ; le cobalt métallique a une pureté de 99,9 %, dans laquelle la teneur en oxygène est inférieure à 500 ppm et la teneur en azote est inférieure à 70 ppm.

2. Procédé selon la revendication 1, dans lequel le bloc d'alliage dans l'étape S1 a une granulométrie de 10-50 mm, telle que déterminée à l'aide de tamis.

3. Procédé selon l'une quelconque des revendications 1 à 2, dans lequel la trempe rapide de la solution d'alliage dans l'étape S2 est réalisée dans des conditions de : régulation d'un débit d'introduction du gaz inerte de 0,4-1,0 m³/min, et maintien d'une pression de 400-1900 Pa.

4. Procédé selon l'une quelconque des revendications 1 à 3, dans lequel la poudre magnétique dans l'étape S3 a une granulométrie de 45-380 µm, telle que déterminée à l'aide de tamis.

5. Procédé selon l'une quelconque des revendications 1 à 4, dans lequel le traitement thermique de cristallisation dans l'étape S4 est réalisé à une température de 630-700 °C pendant 9-18 min.
